

# UNITED STATES PATENT OFFICE.

FREDERICK W. HAINES, OF TOWNSHIP OF SANDWICH EAST, ONTARIO, CANADA, AND  
FRANK L. SORENSEN, OF DETROIT, MICHIGAN, ASSIGNEES, BY DIRECT AND MESNE  
ASSIGNMENTS, TO THE METAL PROTECTION LABORATORY, OF DETROIT, MICH-  
IGAN, A CORPORATION OF MICHIGAN.

## PROCESS FOR DEPOSITING A METALLIC COATING ON VARIOUS METAL ARTICLES OR OBJECTS.

1,397,514.

Specification of Letters Patent. Patented Nov. 22, 1921.

No Drawing.

Application filed September 28, 1918. Serial No. 256,123.

To all whom it may concern:

Be it known that we, FREDERICK W. HAINES, a citizen of the United States, residing in the township of Sandwich East, Province of Ontario, Dominion of Canada, and FRANK L. SORENSEN, a citizen of the United States, and a resident of Detroit, in the county of Wayne and State of Michigan, have invented a new and useful Process for Depositing a Metallic Coating on Various Metal Articles or Objects, of which the following is a full, clear, and exact description.

This invention relates to the coating of metal articles or objects with metal and is applicable to the deposition of thin films of numerous metals upon numerous other metallic bodies, as is frequently desirable for decorative purposes and for the prevention of oxidation, corrosion or rusting.

The objects of our invention are:—The provision of a new and improved process for the deposition, on metallic articles or objects, of a thin film of various metals, which film cannot be peeled or stripped therefrom; which will provide a protective coating on the said metal articles or objects whereby they will be protected against the action of moisture or other rusting influences; and which film can be deposited in a very short time and with the maximum of certainty and the minimum of expense. Other objects of our invention concern the provision of new and useful compositions of matter or working solutions for use in the formation of such coatings, while further objects and advantages of our invention will become apparent as this description proceeds.

The essence of our invention consists in the deposition of the metal in question, from a solution of the same, upon a second metal, by the substitution of a third metal in the solution, and an important feature of our invention is the method employed for restraining and regulating the depositing action so that the film may be closely adherent, fine grained, dense and impervious.

It has long been known that certain metals when immersed in solutions of the salts of other metals will replace those other metals

in the solution with a reduction of the latter to the metallic state. This tendency for one metal to replace another in solution of its salts depends upon the electrolytic condition of those metals with respect to each other, usually expressed as electrolytic potential or electrolytic solution pressure. In the following table based upon recent authorities, the more common metals are arranged in the order of their electrolytic potential, beginning with the most positive:

|            |              |
|------------|--------------|
| Magnesium, | Lead,        |
| Aluminum,  | Tin,         |
| Manganese, | Copper,      |
| Zinc,      | Hydrogen, 65 |
| Cadmium,   | *Arsenic,    |
| Iron       | *Bismuth,    |
| Cobalt,    | *Antimony.   |
| Nickel,    |              |

\*Order uncertain.

In general a metal will replace, from a solution of its salts, any other metal of lower electrolytic potential, unless the difference between the potentials is small. The replacement is also influenced by the relative concentrations of the different metallic ions in the solution. Little or no commercial value has hitherto attended this knowledge, since the metallic deposits so obtained have always been soft, pervious, spongy, friable and imperfectly adherent, thus possessing neither decorative nor protective qualities.

It has also been known that when certain pairs of metals are immersed into a solution of the salt of some metal which is more negative than one at least of the first metals, the metal in solution is ordinarily deposited upon both metal bodies; we have discovered that by the employment of proper methods this deposition can be limited to the surface of the more negative metal and can be rendered so hard, tough, impervious and adherent so as to possess both decorative and protective qualities of a high order.

In order to accomplish this result we employ a solution containing a very low concentration of the metal or metals to be de-

posed. This is most conveniently effected by using a saturated solution of some very slightly soluble compound of the metal to be deposited, the saturation of the solution being maintained by the presence in the solid form of an excess of this compound in contact with the liquid. We also ordinarily employ in the solution a quantity of some acid which shall energize the same but without materially increasing the solubility of the essential compound or independently attacking the anode metal to any appreciable extent.

As a concrete example, suppose it be desired to deposit metallic tin upon the surface of an iron article, we have found the following to be a good bath:

|                                                        |             |
|--------------------------------------------------------|-------------|
| Tin phosphate, $\text{Sn}_3(\text{PO}_4)_4$            | 2 ozs.      |
| Zinc oxid, $\text{ZnO}$                                | 2 ozs.      |
| Ortho-phosphoric acid, $(\text{H}_3\text{PO}_4$ , 85%) | 1 fluid oz. |
| Water (to make)                                        | 1 gal.      |

This bath is preferably used at or near the boiling point and the iron article is merely immersed therein in contact, either direct or indirect, with the replacing metal, ordinarily metallic zinc. The purpose of the zinc oxid is to act as a restrainer by regulating the acidity of the solution. It is equally possible to add the zinc salt in the form of zinc phosphate with a corresponding reduction in the phosphoric acid added. The tin salt dissolves very sparingly and at the same rate as used. The main advantage of the heating is to keep the contents of the bath thoroughly stirred by the ebullition and convection currents although it also has other advantages.

Deposition upon the iron will begin immediately and will afford a beautiful, frosted, solid, adherent coating of metallic tin, extremely resistant to atmospheric or salt conditions. While the coating may be sufficiently thick for some purposes at the end of a few minutes, such as five minutes, we prefer for most purposes to allow the action to go on for from ten minutes to an hour or more. The size of the article also has some effect, massive articles generally taking a rather longer time than smaller ones; however our invention is independent of the length of time employed since a usable coating will be produced very promptly while an increase in the thickness thereof will proceed for a considerable time.

Other compounds than those of zinc can be used in the solution provided they be compounds of metals which the anode substance will not reduce to the metallic form. For example, magnesium oxid or aluminum hydroxid can be employed with equal facility although we prefer the zinc.

In case we desire to deposit a coating of lead upon a ferrous metal article we have

successfully employed the following formula:

|                            |        |
|----------------------------|--------|
| Lead oxid, $(\text{PbO})$  | 2 ozs. |
| Zinc oxid, $(\text{ZnO})$  | 2 ozs. |
| Ortho phosphoric acid, 85% | 1 oz.  |
| Water                      | 1 gal. |

The ferrous metal article is immersed in the solution (preferably heated to or near the boiling point) in contact, either direct or indirect, with a more positive metal such as a piece of metallic zinc. The deposit in this case is of darker color than the tin but is equally firm, adherent, and fine grained.

In case we desire to deposit a coating of nickel upon a ferrous metal article we have successfully employed the following solution:

|                       |        |
|-----------------------|--------|
| Nickel phosphate      | 2 ozs. |
| Zinc oxid             | 2 ozs. |
| Ortho-phosphoric acid | 1 oz.  |
| Water (to make)       | 1 gal. |

The iron article is immersed in the solution in contact with a piece of zinc as before.

Furthermore by our invention we are able to effect deposition upon metals other than iron. Thus we are able to deposit upon one coating an additional layer or layers of other metals provided that the same be more negative than the anode substance. For example, after having subjected the ferrous metal article, in contact with zinc, to the action of the lead-containing solution above described, the same can be subjected to the action of a tin-containing solution, and a very perfect coating of tin deposited thereon, with corresponding increase in decorative and protecting effect; or after having subjected the ferrous metal article, in contact with zinc, to the action of any of the solutions above named, the same may be subjected to the action of a solution containing one of several other metals, such as antimony, whereupon an additional coating of that other metal will be secured.

In fact we are able by our invention to deposit simultaneously upon the iron article a plurality of different metals. For example in order to coat iron with lead and tin simultaneously we have employed with satisfactory results the following solution:

|                 |        |
|-----------------|--------|
| Tin phosphate   | 1 oz.  |
| Lead oxid       | 1 oz.  |
| Phosphoric acid | 1 oz.  |
| Water (to make) | 1 gal. |

The iron article is immersed in the solution (preferably heated) in contact with a piece of zinc as before. The resulting coating possesses a thickness and impermeability apparently superior to any coating obtainable with either metal alone. In this solution the lead oxid appears to have the same action as the zinc oxid of previous formulæ.

- so far as regulating the action is concerned; but with this difference that owing to its more negative character it is reduced to the metallic form.
- 5 As another example of the deposition of a compound coating we find it possible and frequently desirable to deposit a coating of antimony in conjunction with the other metals heretofore mentioned. For the deposition of a combined coating of tin and antimony the most successful bath we have yet discovered is the following:
- Tin phosphate (or hydroxid),  
 $\text{Sn}_3(\text{PO}_4)_2$  2 ozs.
- 15 Zinc chlorid,  $\text{ZnCl}_2$  2 ozs.
- Boric acid,  $\text{H}_3\text{BO}_3$  2 ozs.
- Antimony oxid,  $\text{Sb}_2\text{O}_3$  40 grains.
- Water (to make) 1 gal.
- 20 In order to deposit a combined coating of lead and antimony, or nickel and antimony, we merely substitute for the tin phosphate in the above formula an equal quantity of lead oxid or of nickel phosphate (or oxid).
- 25 The compound coating thus obtained is thicker, more adherent, and more resistant chemically than we have obtained from the other formula.
- Any one of the coatings can be deposited upon brass or copper articles in the same manner as upon iron; and other anodes than zinc can be employed for example, aluminum, which we have used with considerable success for some purposes or magnesium, which is still more positive. The solution tendency can, if desired, be accelerated, restrained, or otherwise modified, by the application of electric potential externally derived.
- 30 It will be understood that we do not limit ourselves to the metals mentioned, since other metals in the replacement series can be employed within the scope of our invention, either singly, simultaneously, or successively. We do not restrict ourselves to the use of only the particular salts herein suggested or enumerated. And we do not restrict ourselves to the use of the particular restrainers herein set forth, or even to any restrainer whatever; since in instances where restrainers are desirable it is possible to employ other than zinc compounds.
- 35 Having thus described our invention, what we claim is:—
1. The process of coating metal articles by replacement in a solution of the desired coating metal, which contains the step of restraining the deposition by placing in the solution an oxid, which in this process is not reduced to its metallic form.
2. The process of protecting corrodible metal articles which consists in depositing thereon simultaneously a plurality of more negative metals at a temperature less than the melting point of any of said metals. 65
3. The process of coating a metal with a second metal which consists in immersing the first metal, in contact with a third metal more positive electrically than either of the first metals, in a saturated solution of some compound of the second metal which is only slightly soluble, and meanwhile maintaining in contact with said solution an excess of such slightly soluble compound 70
4. The process of protecting corrodible metal articles which consists in depositing thereon a plurality of layers of metals each more negative than the last. 75
5. The process of treating ferrous metal articles which consists in immersing the same, in contact with zinc, in a weak solution of an oxygen compound of one or more metals lying between iron and hydrogen in the electrolytic potential series, together with a small amount of the oxid of some metal lying upon the opposite side of hydrogen in said series. 80
6. The process of treating ferrous metal articles which consists in immersing the same, in contact with zinc, in a weak solution of an oxygen compound of one or more metals lying between iron and hydrogen in the electrolytic potential series, together with a small amount of oxid of antimony. 85
7. The process of surface treating ferrous metal articles which consists in immersing the same, in contact with zinc, in a solution containing the phosphate of one or more metals lying between iron and hydrogen in the electrolytic potential series together with a small amount of an oxid of some metal lying upon the opposite side of hydrogen in said series. 95
8. The process of surface treating ferrous metal articles which consists in immersing the same, in contact with zinc, in a solution containing the phosphate of one or more metals lying between iron and hydrogen in the electrolytic potential series, together with a small amount of antimony trioxid. 105
9. The process of treating ferrous metal articles which consists in covering the same with a coating consisting of or containing antimony, or a metal adjacent thereto in the electrolytic potential series. 110
- In testimony whereof, we hereunto affix our signatures.

FREDERICK W. HAINES.  
 FRANK L. SORENSEN.